

# UNITED STATES PATENT OFFICE.

ISAAC TYSON, JR., OF BALTIMORE, MARYLAND.

## IMPROVEMENT IN MANUFACTURE OF CHROMATE OF POTASH.

Specification forming part of Letters Patent No. 4,224, dated October 9, 1845.

*To all whom it may concern:*

Be it known that I, ISAAC TYSON, Jr., of the city of Baltimore, in the State of Maryland, manufacturing chemist, have made a new and useful Improvement in the Manner of Manufacturing the Salt known under the Name of "Chromate of Potash;" and I do hereby declare that the following is a full and exact description thereof.

My improvement in this process consists in the use of a large proportionate quantity of wood-ashes as a substitute for its equivalent of the carbonate of potash or other alkaline salt; and this substitution is not made for the mere purpose of lessening the quantity of the alkaline salts of commerce, which it may be necessary to employ, but I have proved by careful experiment that a larger quantity of the chromate is obtained from a given weight of the ore when wood-ashes are thus used than when the whole of the alkali is supplied by the salts of commerce, the foreign matters contained in the wood-ashes manifestly producing this effect. In other respects the process is managed as heretofore—that is to say, the ma-

terials are pulverized and then intimately mixed with the wood-ashes. The proportion of the respective ingredients will of course vary with their purity, which the manufacturers must ascertain by the usual modes. The proportions which I have generally found to answer well are one part, by weight, of the chrome ore and of the alkaline salt, and one and a half part, by weight, of the ordinary wood-ashes. I will observe, however, that in my improved process I have found that the heat may be increased with advantage.

Having thus fully described the nature of my improvement in the process of manufacturing the salts of chrome, what I claim therein as new, and desire to secure by Letters Patent, is—

The using of wood-ashes in mixture with the chrome ore and with the alkaline salt, for the purpose and in the manner herein fully set forth.

ISAAC TYSON, JR.

Witnesses:

WM. M. JITTON,  
LLOYD NORRIS.